

Sept. 30, 1930.

B. P. FINKBONE

1,776,852

PROCESS OF GALVANIZING SHEET METAL

Filed Nov. 30, 1925



INVENTOR.  
Benjamin P. Finkbone  
BY *Allen & Allen*  
ATTORNEYS

## UNITED STATES PATENT OFFICE

BENJAMIN P. FINKBONE, OF MIDDLETOWN, OHIO, ASSIGNOR TO THE AMERICAN ROLLING MILL COMPANY, OF MIDDLETOWN, OHIO, A CORPORATION OF OHIO

## PROCESS OF GALVANIZING SHEET METAL

Application filed November 30, 1925. Serial No. 72,138.

My invention relates to the problem of coating a piece of sheet metal with commercially pure zinc coating. So far as I am aware no one in the past has accomplished this, and I find that a thicker coating of pure zinc can be imposed upon the surface of a piece of sheet metal, than is practical in the instance of the usual impure spelters in general use today, because the pure zinc appears to be more tightly adherent, and more ductile so as to permit the sheet to be worked up, corrugated or formed without loosening or cracking the coating. By pure zinc or commercially pure zinc I refer to either electrolytic zinc or to commercially available zinc that is insufficiently alloyed to be distinct therefrom in its properties.

I have found that the necessary temperatures employed in maintaining a bath of pure zinc in proper molten condition, in order to properly coat a piece of sheet metal, are sufficiently higher than those called for in the usual galvanizing processes, to require a different mode of procedure.

In the first place the flux must be of a particular type, which, although known in the arts, has not been advanced for use under high temperatures so far as I am advised.

In the next place the highly heated flux and the zinc in the presence of the iron body of a flux box, results in so much zinc and iron alloy, that the same renders the process impossible, due to this alloy or "dross" collecting on the surface of the zinc and spotting the sheet, and this has to be avoided by lining the flux box with a material which will not react with the metal or the flux.

In the third place, I have found it desirable to control the temperature in the flux box which will serve to maintain a proper flux bath at the zinc temperatures called for when using pure zinc, with some mode of applying heat in addition to those ordinarily employed.

Finally in removing the sheet from the zinc pot, after it has passed down through the flux box, and is then to be drawn out through the "exit rolls", I find it necessary to provide a particular mode of preventing the rolls from carrying flux in spots onto the sheets.

The usual mode of cleaning the exit rolls with a body of flux, will not serve for the reason that the high temperatures called for, make the cleansing flux or sal-ammoniac so liquid that it will carry around on the rolls. This as has been stated, spots the sheets. By using a body of some inert substance such as sand, to wipe the exit rolls, and a particularly moist sal-ammoniac imposed on the top of the sand so as to contact with the rolls, I provide for clean rolls, and still keep the rolls in proper condition of coating with molten zinc.

While I have devised preferred mechanism for accomplishing the various steps of my process, still inherently it is a novel process of treating a piece of sheet metal and in this application I propose to state the steps of treatment as independent of mechanism.

I have illustrated in the drawing a preferred mechanism for accomplishing my purpose, in which:

The figure is a central longitudinal section of an apparatus for carrying out my invention.

The equipment for use with my novel galvanizing process follows the usual lines of construction in sheet metal galvanizing except for several details of structure. Thus I have shown the kettle 1, set in suitable brick-work 2. Arranged to be driven within the kettle are the bottom rolls 3, and extending from the receiving end of the kettle to the bottom rolls and from thence to the exit rolls 4, are the curved guides 4<sup>a</sup>, which define the path of movement of a piece of sheet metal, same being inserted into the guides, fed along by the bottom rolls, and finally grasped by the exit rolls and fed out of the kettle.

The kettle is heated by suitable burners 5, in the instance shown being gas burners arranged around the kettle. A hollow rectangular casing 6 formed of metal lined with fire clay or fire bricks is suitably supported at the receiving end of the kettle, and in connection with whatever type of cover is used for the kettle, there will be provided a baffle bar 7 located close to the exit rolls 4 on the side toward the body of the kettle.

The casing 6 is the flux box, and as has been

noted, in my process, the box must be lined with material highly resistant to heat and chemical action. Also I have provided the flux box with a hollow outer wall leaving space 8 in which is set a gas burner 9.

In use the kettle is filled with molten zinc, in my process the commercially pure zinc being used instead of an alloy as is customary in galvanizing sheet metal. The zinc is kept 10 in molten condition by the gas burners.

Within the flux box, which dips below the surface of the zinc, is placed the flux which melts and floats on the surface of the zinc and is held in place by the flux box. As a flux 15 I find that a mixture of zinc ammonium chloride and ammonium chloride accomplishes the required purpose of providing the proper surface cleaning under the particular conditions as to nature of molten metal and required temperatures involved.

To state the exact proportions of these two substances would possibly mislead more than assist those skilled in the art, because the amount of cleaning required on the sheet 20 metal is dependent upon how effective has been the prior pickling or other cleansing action. I use a flux formed of 60% ammonium chloride and 40% zinc ammonium chloride, which I find gives the best results, but increase of the amount of ammonium chloride 25 might be required for unclean sheets. Naturally zinc ammonium chloride will develop in the flux after its use has been started and this should be taken into account.

The theory of flux action is more or less 30 a matter of speculation, and in practice the requirements are the prevention of flux adhering to the sheet, proper cleaning action, and minimum loss of spelter, through chemical action.

In order to provide the high heat necessary 35 for the flux, I use the additional burner in the flux box wall, or insert a special double walled box into the flux box for providing the additional gas flame, or equivalent source of heat.

At the exit rolls I provide a sufficient 40 amount of sand of high grade (ordinarily river sand will not serve), which is floated on the zinc between the inner exit roll and the baffle bar, and the outer exit roll and the kettle wall as indicated at 11. On top of the sand I place ammonium chloride (sal ammoniac) as at 12, which I keep wet with 45 proper spraying, with water. This arrangement at the exit end of the kettle keeps the exit rolls well plated with molten zinc, and still keeps them clean by the action of the flux followed by the scrubbing action of the sand, which is in moist condition also due to the moisture of the flux.

As a process, my invention could be well used with other equipment, the requirements 50 being the proper treatment for the exit rolls, 55 and the properly fluxed entrance of the sheets

into the bath, with the added heat used, and the special flux protected by materials which will not react chemically at the high temperatures, causing a dross on the zinc surface.

This mode of procedure is to be contrasted 70 with the usual one in galvanizing sheets in which the flux on the exit rolls merely floats there and is not so liquid as to be carried around with them.

A sheet of material coated with zinc using 75 the mode of procedure outlined, has been found to have a smoother and denser coat and one more adherent to the metal. The chance of deterioration by corrosion and abrasion is rendered less likely, and the chance of the 80 coating being broken in working up the galvanized sheet is much reduced. Thus while in ordinary practice about 2 ounces of zinc per square foot can be applied to a piece of sheet steel or iron, by my process a 3 to 3 1/4 85 ounce coating may be applied to a like unit of area, and the working properties will be just as good. The custom of the trade calculating zinc coating is as follows:—As an instance, a sheet 2 feet wide by 2 feet long 90 would be considered as having four square feet, and a two ounce coating would consist of eight ounces of zinc on the above dimensioned sheet. It is a physical fact that there 95 are eight square feet of surface of the instanced sheet, but the custom of the trade with reference to coatings is to designate it as having four square feet.

By thickness of coating I provide for longer 100 life and less chance of destruction by abrasion and the like, and by pureness of coating I cut down the chances of loss by normal processes of corrosion to which galvanized metal is subjected.

What I claim as my invention, is—

1. In a process of galvanizing sheet metal, 105 wherein the sheet metal is drawn by rolls through a bath the steps which consist in using as a bath molten zinc substantially free of impurities, or alloying elements, and 110 keeping said rolls clean by a body of inert abrasive substance in finely divided form, such as sand, on the top of which is supported a body of moistened flux through which the rolls wipe.

2. In a process of galvanizing sheet metal, 115 wherein the sheet metal is drawn by rolls through a bath, the steps which consist in using as a bath molten zinc substantially free of impurities or alloying elements, floating 120 a body of flux on the zinc where the sheet enters the same, protecting the flux by an inert surrounding body to prevent formation of dross, and keeping said rolls clean by a body of inert abrasive substance in finely 125 divided form, such as sand, on the top of which is supported a body of moistened flux through which the rolls wipe.

3. In a process of galvanizing sheet metal, 130 wherein the sheet metal is drawn into a bath,

the steps which consist in using as a bath molten zinc substantially free of impurities or alloying elements, floating a body of flux on the zinc where the sheet enters the  
5 same, said flux containing zinc ammonium chloride, protecting the flux by an inert surrounding body to prevent formation of dross, applying heat to the zinc to maintain it in molten condition, and keeping said rolls clean  
10 by a body of inert, abrasive substance in finely divided form, such as sand, on the top of which is supported a body of moistened flux through which the rolls wipe.

BENJAMIN P. FINKBONE.

15

20

25

30

35

40

45

50

55

60

65